

March 15, 1960

B. LEOPOLD ET AL

2,928,825

CATALYSIS OF THE AGEING OF ALKALI CELLULOSE

Filed Sept. 2, 1958



1

2,928,825

## CATALYSIS OF THE AGEING OF ALKALI CELLULOSE

Bengt Leopold, Donald B. Mutton, and William R. Saxton, all of Hawkesbury, Ontario, Canada, assignors to Canadian International Paper Company, Montreal, Quebec, Canada, a corporation of Canada

Application September 2, 1958, Serial No. 758,446

8 Claims. (Cl. 260—233)

This invention relates broadly to the depolymerization of cellulose. More particularly, the invention is concerned with the catalytic ageing or depolymerization of alkali cellulose obtained from various cellulosic materials such as wood, refined cotton, etc., to decrease its viscosity. The invention finds its greatest application in the viscose process for producing rayon by providing improvements in the ageing of the alkali cellulose in viscose manufacture. The invention is also of particular value in ageing or depolymerizing alkali cellulose for production of cellophane, cellulose ethers, or any other cellulosic products in the manufacture of which alkali cellulose is an intermediate product.

The manufacture of viscose rayon and cellophane employs solutions of cellulose. In order to obtain solutions of low enough viscosity to handle conveniently, the molecular weight of the cellulose must be reduced considerably from its original value in the wood, cotton or other cellulosic material from which it is obtained. This cellulose depolymerization is carried out mainly in the case of wood during the cooking of the wood, the bleaching of the pulp, and the ageing of the alkali cellulose. Depolymerization by bleaching is expensive to the pulp manufacturer since it consumes large quantities of chemicals which are not inexpensive and it reduces yield. Ageing of alkali cellulose may require a considerable length of time and it is expensive and inefficient for the rayon manufacturer to increase that time. If the rate of depolymerization during ageing could be increased sufficiently, then all or most of the degradation now carried out during the bleaching and ageing steps could be performed during the ageing period alone, and even the ageing time could be reduced. This would enable the rayon manufacturer to save time and reduce costs and the pulp manufacturer to reduce chemical costs as well as to sell higher viscosity pulps which might yield improved rayon yarn and cord.

It is known that the transition metals, such as iron, manganese and cobalt, particularly the latter, catalyze the ageing of alkali cellulose. The prior art is limited to employing water-soluble and alkali-soluble compounds of these metals. These compounds are particularly soluble in steeping caustic, especially in the presence of hemi-cellulose. It is general practice to employ caustic solutions containing between about 17 and 25% by weight of caustic soda as a steeping liquid. To effect necessary economy it is essential to reuse the caustic steeping solutions for treating subsequent batches of pulp. When the transition metal catalyst is relatively soluble in the steeping alkali, variable amounts of the catalyst are retained by the steeping liquid when separated from the alkali cellulose. This leads to large variations in ageing reactivity imparted to the alkali cellulose subsequently produced with the result that viscosity control is difficult. This is especially true in the case of cobalt compounds which are much more active catalysts than compounds of manganese or iron.

We have discovered that in accordance with the present

2

invention certain organic complexes or chelate compounds of cobalt are not only substantially completely insoluble in water and steeping caustic, but what is more important and unexpected, these complexes retain the ability to catalyze the ageing of alkali cellulose. These alkali-insoluble complexes not only catalyze the ageing of alkali cellulose, but they are retained by the alkali cellulose and do not contaminate the steeping caustic. Consequently, the present invention makes it possible to effectively catalyze the ageing of the alkali cellulose without contaminating the steeping caustic, thereby permitting reuse of the steeping caustic without the concomitant variations in ageing reactivity which have plagued the prior art. Since the steeping caustic, after separation from the cellulose, contains substantially no catalytic cobalt complex or chelate compound, it can be reused with the next batch of cellulose to which an exact amount of catalyst has been added to produce controlled ageing of the cellulose. During the research investigation which resulted in the present invention it was found that only certain organic complexes or chelate compounds of cobalt are substantially insoluble in steeping caustic and yet retain the ability to catalyze the ageing or depolymerization of alkali cellulose.

15 The process of the invention provides greater control over the degree of an rate of depolymerization. This control is important since too much depolymerization results in weakened rayon fiber strength.

20 It is an object of the present invention to provide improvements in the depolymerization of cellulose.

25 It is also an object of the present invention to provide an improved process for the controlled depolymerization of cellulose in the manufacture of viscose rayon and cellophane.

30 It is a further object of the present invention to provide organic coordinate compounds or complexes of cobalt which are substantially insoluble in steeping alkali and yet catalyze the ageing of alkali cellulose and which do not contaminate the steeping alkali.

35 The foregoing objects, as well as others, will be apparent to those skilled in the art from the present description, taken in conjunction with the accompanying coordinate diagram illustrating the effect of varying amounts of one of the cobalt complex catalysts on the ageing of alkali cellulose.

40 In accordance with the process of the present invention for depolymerizing cellulose, a small amount of an alkali-insoluble cobalt complex or coordinate compounds as hereinafter defined is brought into the presence of cellulose, such as wood pulp, and steeping alkali to catalyze cellulose depolymerization. Since such processes as the viscose process and the manufacture of cellulose ethers involve conversion of cellulose into alkali cellulose, usually by steeping sheets of cellulose in an aqueous caustic soda solution containing from about 17 to 25% of caustic soda, it is desirable for use in that process to add the cobalt complex catalyst to the cellulose prior to the steeping operation. After the cellulose has been steeped sufficiently in the alkali to substantially convert the cellulose to alkali cellulose, the alkali cellulose is separated from the steeping alkali by draining and pressing. The alkali cellulose, after comminution, is permitted to age until the desired degree of depolymerization has been attained. The aged alkali cellulose is then in condition for xanthation and conversion to viscose in accordance with well established procedures or it may be employed for other desired purposes which require aged or depolymerized alkali cellulose.

45 Additions of the cobalt complexes to the cellulose may be made by any suitable method. In one preferred method of application a dilute aqueous suspension of the

50

55

60

65

70

cobalt complex is sprayed or striped on to the formed pulp sheet as it passes into the drier on the pulp machine or into the cutter. Alternatively, dilute solutions of the cobalt complexes in an organic liquid, such as chloroform, may be employed. In accordance with another method, the cobalt complex may be formed *in situ* on the cellulose by adding a soluble salt of cobalt, such as cobalt chloride, with the insolubilizing organic complexing agent, the latter being added in excess of the stoichiometric amounts necessary to react with and complex substantially all the cobalt chloride.

Although any amount of cobalt complex catalyst may be added to the cellulose, it is usually necessary to add only very small amounts, because of the high catalytic activity of these complexes. In addition, we have found that increasing the amount of cobalt catalyst added to the cellulose has progressively less effect on the rate of ageing, so that normally there is little additional advantage in adding more than 5 p.p.m. of cobalt on the weight of bone dry cellulose. Similarly there is no lower limit to the amount of cobalt catalyst which may be applied to the cellulose. We have found, however, that the lower the catalyst concentration, the more sensitive is the rate of ageing to small variations in the catalyst concentration. For these reasons, we usually prefer to employ between 0.5 and 3 p.p.m. of cobalt on the weight of bone dry cellulose. As those skilled in the art will recognize, the optimum amount of catalyst will vary somewhat depending upon the original pulp viscosity and the desired viscosity of the aged alkali cellulose, as well as time and temperature of ageing.

It is well known that cobalt forms coordinate compounds or complexes with a wide variety of anions and neutral molecules. The essential feature of a coordinated group is that it contains an electron pair which it can share with the metal ion in the formation of a more or less covalent bond. Cobalt usually has a coordination number of 6 and can thus form 6 essentially covalent bonds with coordinated groups. In the case of simple cobalt salts, the coordinated groups are usually water molecules, 6 in number. The cobalt complexes of the present invention are formed with bifunctional organic reagents which form more than one covalent bond with the cobalt ion. When the positive charges of the cobalt ion have been neutralized by coordinate groups, the resulting complex is electrically neutral and is no longer an electrolyte. These characteristics of the cobalt complexes of the present invention are responsible for their insolubility in water and alkaline solutions.

The cobalt ion is capable of existing in the bivalent or trivalent state. In its simple salts, such as the chloride, the cobalt is almost always bivalent. Most complexes or coordinated compounds of cobalt usually occur with a trivalent cobalt ion. The cobalt complexes of the present invention appear to occur as mixtures of the complexes formed by bivalent and trivalent cobalt with the organic complexing agent. While no precise valence can be ascribed to the cobalt in the complex, the complexes of the invention may be characterized in terms of their alkali insolubility and from the fact that they are produced by reacting a water-soluble salt or cobalt, such as cobalt chloride, with a stoichiometric excess of the organic complexing agent.

The cobalt coordinate compounds or complexes suitable for use as catalysts in the invention may be characterized as cobalt xanthates. Desirably they possess the following structural formula:



wherein  $n$  is a number between 2 and 3, R is an alkyl, cycloalkyl or aryl group.

Examples of the cobalt complexes of the invention are the complexes of cobalt with ethylxanthate, butyl-

xanthate, methylxanthate, cyclohexylxanthate and phenylxanthate.

In order more clearly to disclose the nature of the present invention, the following examples illustrating the invention are disclosed. It should be understood, however, that this is done solely by way of example and is intended neither to delineate the scope of the invention nor limit the ambit of the appended claims. In the examples which follow, and throughout the specification, the quantities of materials are expressed in terms of parts by weight, unless otherwise specified, and cobalt concentrations are expressed in terms of p.p.m. of cobalt per weight of bone-dry cellulose.

### EXAMPLE 1

A web of Kipawa Tenacell tire cord grade of sulphite wood pulp was spotted uniformly with a dilute aqueous suspension of the cobalt ethylxanthate complex of Example 7 hereinbelow in sufficient amount to deposit about 3.0 p.p.m. of cobalt on the pulp. The cobalt suspension was of such concentration and the pulp was of such thickness and moisture content that about 10 to 15 drops of the cobalt complex suspension were required per square foot of pulp. The pulp sheets were then air-dried in an atmosphere of 65% relative humidity. The dried pulp was steeped for 45 minutes at room temperature (22° C.) in the customary manner in a caustic soda steeping liquor containing 216.5 gms. of sodium hydroxide per liter of solution and containing also 5 gms. per liter of hemi-cellulose. The resulting alkali cellulose sheets were then drained and pressed to expel the steeping liquor to give a cellulose content of 32%. The sheets were shredded and the alkali cellulose crumbs were aged for 24 hours at 22° C. The crumbs were then xanthated with 39% of carbon disulfide based on the weight of cellulose in the alkali cellulose by reacting for 2 1/4 hours at 26° C. in the absence of air. The resulting xanthate was then mixed with dilute sodium hydroxide solution to give a viscose having a composition of about 7% cellulose and 6% sodium hydroxide. The resulting viscose had a spinning viscosity of 26.1 seconds when measured by the falling ball method. A sample of identical pulp but without the cobalt addition, processed in an analogous manner, required 65% more ageing time to give the same viscose spinning viscosity. The tensile and durability properties of rayon produced from the viscose of the example and of the control were equivalent.

The extent of any contamination of the used steeping caustic by cobalt complex in the example was determined. The caustic drained and pressed from the pulp was reused to steep further batches of control pulp, sufficient fresh caustic being added to replace the caustic taken up by the previous batch of cellulose. Control batches of alkali cellulose employing the used caustic were then aged and made into viscose as described and the spinning viscosity measured. It was found that, when caustic from the batch treated with cobalt complex was reused, the spinning viscosity of the second batch of viscose was substantially the same as that obtained when caustic which had at no time been treated with cobalt complex was used for steeping. This indicated that the cobalt complex catalyst was completely retained by the alkali cellulose and none of the complex contaminated the recovered steeping caustic. On the other hand, when caustic used to steep a batch of pulp containing the same amount of cobalt in the form of cobalt chloride was reused, the spinning viscosity of the viscose was less than half that obtained when caustic from the above example, employing the cobalt complex of the invention, was reused. This indicated the high degree of contamination of the steeping caustic when employing an alkali-soluble cobalt salt, such as cobalt chloride.

### EXAMPLE 2

75. The foregoing example was repeated, except that vary-

ing amounts of cobalt ethylxanthate complex varying from 0 to 5.0 p.p.m. cobalt based upon bone dry pulp were employed and the resulting alkali cellulose was subjected to various ageing periods of from 0 to 64 hours. The degree of polymerization (D.P.) was observed for each of the various amounts of cobalt complex catalyst employed over the various periods of ageing. The results are recorded in Table I below and plotted in the accompanying diagram.

Table I

| Time (hours) | p.p.m. of cobalt on pulp |     |     |     |     |     |
|--------------|--------------------------|-----|-----|-----|-----|-----|
|              | 0                        | 0.5 | 1.0 | 2.0 | 3.0 | 5.0 |
|              | Cellulose, D.P.          |     |     |     |     |     |
| 0            | 775                      | 775 | 775 | 775 | 775 | 775 |
| 8            | 663                      | 568 | 532 | 516 | 474 | 428 |
| 16           | 599                      | 492 | 428 | 404 | 369 | 352 |
| 24           | 532                      | 361 | 322 | 291 | 283 | 276 |
| 32           | 502                      | 378 | 318 | 263 | 238 | 220 |
| 40           | 461                      | 320 | 262 | 230 | 214 | 205 |
| 48           | 422                      | 302 | 284 | 225 | 205 | 195 |
| 56           | 404                      | 262 | 239 | 207 | 195 | 176 |
| 64           | 386                      | 261 | 211 | 195 | 191 | 163 |

## EXAMPLE 3

The procedure of Example 1 was repeated employing the same wood pulp and alkali steeping liquor except that the 3 p.p.m. of cobalt was provided by the cobalt phenylxanthate complex of Example 8 hereinbelow. When the catalyzed alkali cellulose crumbs were xanthated and converted to viscose, it was found that the ageing time was reduced by 60%. When tested, the used steeping liquor was found to be substantially free from cobalt contamination.

## EXAMPLE 4

The procedure of Example 1 was repeated employing the same wood pulp and alkali steeping liquor except that the 3 p.p.m. of cobalt was provided by the cobalt butylxanthate complex of Example 9. When the catalyzed alkali cellulose crumbs were xanthated and converted to viscose, it was found that the ageing time was reduced by 75%. When tested, the used steeping liquor was found to be substantially free from cobalt contamination.

## EXAMPLE 5

The procedure of Example 1 was repeated employing the same wood pulp and alkali steeping liquor except that the 3 p.p.m. of cobalt was provided by the cobalt methylxanthate complex of Example 10. When the catalyzed alkali cellulose crumbs were xanthated and converted to viscose, it was found that the ageing time was reduced by 55%. When tested, the used steeping liquor was found to be substantially free from cobalt contamination.

## EXAMPLE 6

The procedure of Example 1 was repeated employing the same wood pulp and alkali steeping liquor except that the 3 p.p.m. of cobalt was provided by the cobalt cyclohexylxanthate complex of Example 11. When the catalyzed alkali cellulose crumbs were xanthated and converted to viscose, it was found that the ageing time was reduced by 55%. When tested, the used steeping liquor was found to be substantially free from cobalt contamination.

The preparation of the alkali-insoluble cobalt organic complexes employed in the foregoing examples is described in Examples 7-11 which follow:

## EXAMPLE 7

## COBALT ETHYLXANTHATE COMPLEX

Pure potassium ethylxanthate (1.37 gm.), which is commercially available, was dissolved in 100 ml. of water

and mixed with a solution of 1 gm. of sodium carboxymethyl cellulose in 100 ml. of water. To this solution was added, with very vigorous stirring, a solution of 0.41 gm. of cobalt chloride hexahydrate in 50 ml. of water. (The molar ratio of potassium ethylxanthate to cobalt was 5:1 in order to ensure complete reaction of the cobalt.) A very fine green suspension was formed of cobalt ethylxanthate complex. The complex was found to contain 13.6% cobalt. The calculated value for a complex of divalent cobalt was 19.6% cobalt and for trivalent, 14.0% cobalt.

## EXAMPLE 8

## COBALT PHENYLXANTHATE COMPLEX

To a solution of 25 gm. of phenol in 100 ml. of methyl alcohol were added 18 gm. of potassium hydroxide. The mixture was refluxed for half an hour. Carbon disulphide (20 ml.) was added and refluxing was continued on the steam bath for four hours. After standing overnight, the mixture was filtered and cooled. Ether (100 ml.) was added, and the precipitated potassium phenyl xanthate was filtered off. The product was washed with ether and dried in the vacuum desiccator.

The substantially pure potassium phenyl xanthate (1.70 gm.) was dissolved in 100 ml. of water and mixed with a solution of 1 gm. of sodium carboxymethyl cellulose in 100 ml. of water. To this solution was added, with very vigorous stirring, a solution of 0.41 gm. of cobalt chloride hexahydrate in 50 ml. of water. (The molar ratio of potassium phenyl xanthate to cobalt was 5:1 in order to ensure complete reaction of the cobalt.) A very fine green suspension was formed of cobalt phenyl xanthate complex.

## EXAMPLE 9

## COBALT BUTYLXANTHATE COMPLEX

A mixture of 100 gm. of n-butyl alcohol and 18 gm. of potassium hydroxide pellets was refluxed for one hour and the residual solid was removed by decanting. Carbon disulphide (36 gm.) was added slowly and with constant shaking. The mixture was cooled in an ice bath and the potassium butylxanthate which separated was filtered off and washed with several 25 ml. portions of dry ether. The product was dried in a vacuum desiccator over silica gel.

The substantially pure potassium butylxanthate (1.61 gm.) was dissolved in 100 ml. of water and mixed with a solution of 1 gm. of sodium carboxymethyl cellulose in 100 ml. of water. To this solution was added, with very vigorous stirring, a solution of 0.41 gm. of cobalt chloride hexahydrate in 50 ml. of water. (The molar ratio of potassium butylxanthate to cobalt was 5:1 in order to ensure complete reaction of the cobalt.) A very fine green suspension was formed of cobalt butylxanthate complex.

## EXAMPLE 10

## COBALT METHYLXANTHATE COMPLEX

Methyl alcohol (100 ml.) was refluxed with 25 gm. of potassium hydroxide pellets for 30 minutes and the solution was decanted from any undissolved solid. Carbon disulphide (35 ml.) was added slowly with constant shaking. The mixture was cooled in an ice bath and the resulting crystals of potassium methylxanthate were filtered off and washed with dry ether. The product was dried in the vacuum desiccator.

The substantially pure potassium methylxanthate (1.25 gm.) was dissolved in 100 ml. of water and mixed with a solution of 1 gm. of sodium carboxymethyl cellulose in 100 ml. of water. To this solution was added, with very vigorous stirring, a solution of 0.41 gm. of cobalt chloride hexahydrate in 50 ml. of water. (The molar ratio of potassium methylxanthate to cobalt was 5:1 in order to ensure complete reaction of the cobalt.) A very fine green suspension was formed of cobalt methylxanthate complex.

7  
EXAMPLE 11

## COBALT CYCLOHEXYLXANTHATE COMPLEX

Cyclohexanol (100 ml.) was refluxed with 18 gm. of potassium hydroxide pellets for one hour and the solution was cooled and filtered to remove any undissolved solid. Carbon disulphide (28.5 ml.) was added slowly with constant shaking. The mixture was cooled in an ice bath and the resulting crystals of potassium cyclohexyl xanthate were filtered off and washed with dry ether. The product was dried in the vacuum desiccator.

The substantially pure potassium cyclohexyl xanthate (1.67 gm.) was dissolved in 100 ml. of water and mixed with a solution of 1 gm. of sodium carboxymethyl cellulose in 100 ml. of water. To this solution was added, with very vigorous stirring, a solution of 0.41 gm. of cobalt chloride hexahydrate in 50 ml. of water. (The molar ratio of potassium cyclohexyl xanthate to cobalt was 5:1 in order to ensure complete reaction of the cobalt.) A very fine green suspension was formed of cobalt cyclohexyl xanthate complex.

The terms and expressions which have been employed are used as terms of description and not of limitation, and there is no intention, in the use of such terms and expressions, of excluding any equivalents of the features shown and described or portions thereof, but it is recognized that various modifications are possible within the scope of the invention claimed.

What is claimed is:

1. In the ageing of alkali cellulose the improvement which comprises catalyzing the ageing of the alkali cellulose with an alkali-insoluble cobalt coordinate compound comprising a cobalt xanthate complex selected from the class consisting of cobalt complexes of alkyl, cycloalkyl and aryl xanthates.

2. In the viscose process the improvement which comprises ageing the alkali cellulose in the presence of an

alkali-insoluble cobalt coordinate compound comprising a cobalt xanthate complex selected from the class consisting of cobalt complexes of alkyl, cycloalkyl and aryl xanthates.

3. In the ageing of alkali cellulose, the improvement which comprises ageing alkali cellulose in the presence of an organic cobalt complex having the following structural formula:



wherein  $n$  is a number between 2 and 3, R is a member selected from the class consisting of alkyl, cycloalkyl and aryl groups.

4. The improvement in ageing alkali cellulose which comprises ageing the alkali cellulose in the presence of cobalt ethylxanthate complex.

5. The improvement in ageing alkali cellulose which comprises ageing the alkali cellulose in the presence of cobalt phenylxanthate complex.

6. The improvement in ageing alkali cellulose which comprises ageing the alkali cellulose in the presence of cobalt butylxanthate complex.

7. The improvement in ageing alkali cellulose which comprises ageing the alkali cellulose in the presence of cobalt methylxanthate complex.

8. The improvement in ageing alkali cellulose which comprises ageing the alkali cellulose in the presence of cobalt cyclohexylxanthate complex.

## References Cited in the file of this patent

## UNITED STATES PATENTS

|    |           |                  |               |
|----|-----------|------------------|---------------|
| 35 | 2,682,536 | Mitchell         | June 29, 1954 |
|    | 2,768,968 | Reppe            | Oct. 30, 1956 |
|    | 2,841,579 | Villefroy et al. | July 1, 1958  |